

## UNITED STATES PATENT OFFICE

2,347,955

CATALYST AND METHOD FOR PREPARING  
THE SAMEKarl Korpi, Redondo Beach, Calif., assignor to  
Union Oil Company of California, Los Angeles,  
Calif., a corporation of CaliforniaNo Drawing. Application May 28, 1940,  
Serial No. 337,656

11 Claims. (Cl. 252—211)

The present invention relates to catalysts for reducing the olefin hydrocarbon content of hydrocarbon mixtures containing the same, as for example, in the purification of aromatic hydrocarbon solvents by reducing the olefin hydrocarbon content thereof. The invention relates particularly to catalysts for converting naphthene hydrocarbons into aromatic hydrocarbons and also to the conversion of olefin hydrocarbons to paraffinic, naphthenic and aromatic hydrocarbons. The invention also relates to a method for preparing such catalysts. This application is a continuation, in part, of my co-pending application Serial No. 321,983 filed March 2, 1940.

It is known to produce aromatic hydrocarbon solvents by solvent extraction of straight run gasoline particularly those obtained from California or asphalt base crude oils which are relatively free from olefin hydrocarbons. Past attempt to produce aromatic solvents from gasolines obtained by thermal pyrolysis and/or polymerization of hydrocarbons have not been successful principally for the reasons that (1) the available cracked gasolines have not been particularly rich in aromatic hydrocarbons and (2) these cracked gasolines have contained large amounts of olefinic materials. The first objection has been eliminated to a large extent with the advent of catalytic cracking which will make available pressure distillates containing as much as 50% by volume of aromatic hydrocarbons. The aromatic content of these pressure distillates is about three times as high as that of straight run gasolines obtained from Western crudes and some pressure distillates produced by simple thermal means. Thus, cracked gasolines produced by catalytically cracking oils are a particularly rich source of aromatics from which aromatic solvents may be produced.

However, the recovery of the aromatic hydrocarbons from cracked gasoline has been somewhat uneconomical principally due to the presence of olefin hydrocarbons in the cracked gasoline. The solvent extraction of the cracked gasoline for recovery of the aromatics, as for example, with liquid sulfur dioxide, has resulted in the simultaneous extraction of both the olefin and aromatic hydrocarbons. In order to reduce the olefin content of the aromatic extract to what may be considered a satisfactory value, a rigorous and wasteful sulfuric acid treatment has been required. Straight run gasolines containing aromatics are not subjected to this disadvantage since these are relatively free from olefins.

It is an object of my invention to reduce the olefin hydrocarbon content of pressure distillates or other hydrocarbon mixtures which are rich in aromatic hydrocarbons to produce aromatic solvents which are relatively free from olefin hydrocarbons. It is another object to accomplish the recovery of relatively pure aromatic hydrocarbons without resorting to expensive and wasteful treating procedures.

10 It is an object of my invention to reduce the olefin hydrocarbon content of pressure distillates or other hydrocarbon mixtures which are rich in aromatic hydrocarbons to produce aromatic solvents which are relatively free from olefin hydrocarbons. It is another object to accomplish the recovery of relatively pure aromatic hydrocarbons without resorting to expensive and wasteful treating procedures.

10 I have discovered that olefins may be separated from aromatic hydrocarbons by subjecting the aromatic fraction containing the olefins to catalytic treatment at elevated temperatures. Such catalytic treatment results in converting the olefins into non-olefinic materials such as naphthenic, aromatic and paraffinic hydrocarbons so that in the production of aromatic solvents, the non-aromatic materials may be separated from the aromatic hydrocarbons by simple extraction 20 with selective solvents such as liquid sulfur dioxide.

15 The reactions involved in the thermal catalytic treatment are numerous depending upon the character of the stock undergoing treatment and on the conditions of operation. When treating stocks containing olefins, it is believed that a major reaction is in the cyclization of the olefins into cyclo-paraffin hydrocarbons or naphthenes. Another major reaction taking place 25 resides in the formation of paraffin hydrocarbons from the olefins. Another major reaction of great importance is in the formation of aromatic hydrocarbons from either or both the cyclo-paraffin hydrocarbons present in the original stock or produced from the olefin hydrocarbons. In 30 one case, I subjected to the catalytic treatment a hydrocarbon fraction composed of about 80% olefins and 20% paraffins and obtained a resulting product composed of 5% olefins, 15% aromatics, 35 12% naphthenes and 68% paraffins. This indicates that olefins were changed to cyclo-paraffins, paraffins and aromatics during the treatment. In another case, a hydrocarbon fraction composed of approximately 50% aromatics, 30% naphthenes and 20% paraffins was treated by the catalytic process of my invention. The resulting product of the treatment was composed of approximately 80% aromatics and 20% paraffins. The increase in aromatics from 50% to 80% indicates that all of the naphthenes were converted into aromatic hydrocarbons without substantially changing the paraffins present.

45 It is another object of my invention to convert olefin hydrocarbons into paraffin, naphthene and aromatic hydrocarbons by subjecting hydrocar-

bon fractions containing substantial amounts of olefins to thermal catalytic treatment.

It is thus another object of my invention to subject naphthene hydrocarbon fractions to catalytic thermal treatment to transform the naphthene hydrocarbons into aromatic hydrocarbons.

It is a further object of my invention to provide catalysts particularly adapted for carrying out these conversions.

I have further discovered that the process of deolefination results in materially reducing the sulfur content of stocks containing sulfur. In one particular instance, the sulfur content of the feed was reduced from 0.67 to 0.13% with simultaneous olefin reduction in two passages of the stock through the reactor.

The choice of catalysts in my process for the catalytic treatment of hydrocarbons to transform olefins or naphthenes is extremely important. I have found orthophosphoric acid and other forms of phosphoric acid such as tetra, meta and pyro phosphoric acid to be good catalysts. It is preferable to employ a carrier for the catalyst. Carriers which may be used include charcoal, carbondum, coke and like carbonaceous materials, alumina, clay and the like. Neutral carriers as preformed phosphates and other mineral acid salts of metals may be used.

I have found the activated carbons such as wood charcoal, petroleum and metallurgical coke, soft and hard coals and other carbonaceous materials, bone charcoal, sugar and starch charcoals and the like to be superior to the other carriers. I have found activated carbons prepared from nut shells, such as cocoanut, walnut and the like to be particularly effective carriers for the catalyst. An activated carbon of this type is one commercially prepared by the Carbide and Carbon Chemicals Corporation and sold as "Columbia Activated Carbon." This activated carbon is prepared from cocoanut shells by steam oxidation at high temperatures. I have found a catalyst adsorbed on this type carrier to be about 5 to 50 times as effective as the same catalyst adsorbed on ordinary unactivated wood charcoal. The catalytic material is preferably prepared by adsorbing orthophosphoric acid or other phosphoric acids on the carrier particles of suitable size and porosity and heating the mixture to dryness at a temperature of 300-400° F. The amount of catalyst which is adsorbed on the carrier may vary within wide limits depending upon the character of the catalyst and the carrier. With the phosphoric acid catalysts, I have found it desirable to adsorb as much as 50 to 150 ml. of the acid of 75-85%  $H_3PO_4$  concentration on 250 ml. of the granular carrier. I have found that by saturating the carrier with catalyst and then drying the saturated carrier that the catalytic life of the catalyst is greatly increased over that obtained by adsorbing smaller quantities of the catalyst. For convenience in preparing the catalyst, the strength of the catalyst employed should not preferably be less than substantially 50%  $H_3PO_4$ . However, phosphoric acid of as low as 5 or 10% strength may be used.

Using the above catalyst in treating pressure distillates containing about 20% olefins, I have obtained a reduction of 50-60% in olefin content per pass of the pressure distillate vapors over the catalyst while maintaining a temperature of 750-800° F. and atmospheric pressure in the reactor containing the catalyst.

A catalyst which I have found to be superior to straight phosphoric acid is one in which the

phosphoric acid is partially or totally neutralized by means of a caustic alkali, (potassium, lithium and sodium hydroxides). Such a catalyst may be prepared by first adsorbing the phosphoric acid on the carrier particularly on activated carbon and drying the mixture when necessary by gentle heating. The phosphoric acid on the activated carbon carrier is then partially or totally neutralized by adding thereto a caustic solution of alkali. The resulting mixture is again dried, heating to a temperature of 300°-400° F. when necessary to obtain the drying. One advantage in using a phosphoric acid catalyst which has been partially or totally neutralized with alkali is the fact that this catalyst does not volatilize as readily as straight phosphoric acid, thus enabling the catalyst to be used for a considerably longer period of time. Another advantage resides in the fact that this catalyst is less corrosive to the reactor and accessory equipment than the straight phosphoric acid would be.

The above procedure of first adsorbing the catalyst on the carrier, drying, adding the caustic soda and again drying is very important to obtain a catalyst adapted to produce superior catalytic effect. I have found that when the phosphoric acid is first partially or totally neutralized before being adsorbed on the carrier and dried that the resulting catalyst has only a moderate effect in the catalytic process.

Using this catalyst for treating pressure distillate vapors containing 20% olefins, I have obtained a reduction of 70-90% in olefin content in a single pass of the material over the catalyst while maintaining a temperature of 750-800° F. and atmospheric pressure in the reactor. Further reduction in olefin content may be obtained by decreasing the rate of introduction of hydrocarbon to the reactor or by recycling the product of the first passage through the reactor.

In producing the partially neutralized catalyst, I have discovered that the best results are obtained when the phosphoric acid is neutralized with less than one equivalent of the caustic alkali per mol of the acid. I have found the preferred neutralization to be within the range of  $\frac{1}{2}$  to  $\frac{3}{4}$  equivalents per mol of acid. For example, I have obtained olefin reduction to the extent of nearly 90% in a single pass of the olefinic stock through a phosphoric acid catalyst which had been neutralized with  $\frac{1}{2}$  to  $\frac{3}{4}$  equivalents of caustic alkali per mol of the acid. Using straight phosphoric acid catalyst, the reduction in olefin content was about 60% per pass through the catalyst and using phosphoric acid catalyst which had been partially neutralized with  $\frac{3}{4}$  equivalents of the alkali per mol of the acid, the reduction in olefin content of the stock was about 77% per pass. Using phosphoric acid catalyst which had been partially neutralized with one, one and one-half and two equivalents of the caustic alkali per mol of the acid, the catalysts were effective in reducing the olefin contents of stock by approximately 72%, 70%, and 58% respectively. A completely neutralized phosphoric acid catalyst was effective to reduce the olefin content of the stock by only 30%. In the above, the partially neutralized catalyst is prepared as described above.

It is thus another object of my invention to provide a catalyst composed of partially neutralized phosphoric acid on activated carbon in order to transform olefin hydrocarbons into non-olefin hydrocarbons and preferably to provide a catalyst composed of phosphoric acid adsorbed on ac-

tivated carbon, the phosphoric acid being neutralized with approximately  $\frac{1}{6}$  to  $\frac{2}{3}$  equivalents of caustic alkali per mol of the acid.

Another catalyst which I have found to be superior to straight phosphoric acid and even better than the partially or totally neutralized phosphoric acid adsorbed on activated carbon is one composed of silica contained on activated carbon or silicic acid adsorbed on the activated carbon. Such a catalyst may be prepared by first adsorbing an aqueous sodium silicate solution on the granules of activated carbon and then treating these granules containing the adsorbed sodium silicate solution with hydrochloric acid in order to precipitate silicic acid on the granules. Other acids such as sulfuric, acetic, phosphoric, nitric, carbonic, etc., which are stronger than silicic acid and which therefore liberate free silicic acid from silicates may be used in the place of the hydrochloric acid. The granules are then thoroughly washed with water in order to remove any free hydrochloric acid and sodium chloride that may have been formed. The thus treated granules are then dried at a temperature of about 300° F. in order to remove water. This drying causes part of the silicic acid to be converted into silica, the remaining silicic acid being converted into silica during the course of a few minutes of catalytic operation at the more elevated temperatures of about 800° F. The catalyst thereafter may be said to consist of silica contained on the activated carbon carrier.

Using this catalyst for treating pressure distillate vapors containing 44% olefins, for example, I have obtained a reduction of 80-90% in olefin content in a single pass of the material over the catalyst while maintaining a temperature of about 750-800° F. and atmospheric pressure in the reactor.

In preparing the catalyst, the sodium silicate solution which is generally purchased as a thick syrup is preferably first diluted to a thin consistency with 2 to 4 parts of water. Then a sufficient amount of the solution is adsorbed on the activated carbon carrier as to incorporate about 20 to 30% of the undiluted sodium solution. The granules are then treated with hydrochloric acid preferably 3N-HCl which is accomplished by soaking the granules in about two volumes of the acid for several days. The excess acid is then drained from the granules which are then washed thoroughly with water and dried.

It is thus another object of my invention to provide a catalyst composed of silicic acid or silica adsorbed on activated carbon. It is another object of the invention to prepare this catalyst by adsorbing sodium silicate solution on activated carbon and then treating the activated carbon carrier with hydrochloric acid to convert the sodium silicate to silicic acid and then heating the thus treated silicic acid on the carrier to convert part or all of the silicic acid to silica.

I have found that the presence of moisture during the reaction aids materially in prolonging the catalytic activity of the catalyst used in the process of treating hydrocarbons particularly when using catalyst of the phosphoric acid type. I have observed that the presence of moisture in the reactor has prolonged the life of the catalyst more than 40 hours without materially decreasing the ability of the catalyst to convert the olefins or naphthenes contained in the charging stock whereas without moisture, the catalyst showed signs of loss in activity after only a few

hours operation. The moisture may be introduced into the catalytic zone by merely injecting water into a preheater through which the vaporized charging stock is passing on its way into the catalytic reactor. The heat in the vapors and in the preheater vaporizes the water which then passes through the reactor in the form of steam which may be removed from the treated vapors by condensation. The high temperature employed in the reactor causes a part of the phosphoric acid to be volatilized and removed together with the treated hydrocarbons and steam. This will be recovered with the condensed water which may be recycled to the reactor.

While the above are the preferred catalysts, other catalysts which may be used to transform olefin or naphthenes in hydrocarbon mixtures comprise zinc, cadmium and other metal phosphates, hydroxides or alkali and alkaline earth metals such as sodium, potassium, lithium and calcium hydroxides, metal halides such as zinc, aluminum and iron chloride and bromides, metal sulfates such as sodium, potassium and zinc sulfate and oxides of metals and non-metals such as aluminum and boric oxides. The catalysts are preferably used with activated carbon carriers. In general, any catalyst which has heretofore been employed for the purpose of polymerizing gaseous hydrocarbons may be used as a catalyst in the process of deolefination of hydrocarbons forming the subject matter of my invention.

The temperature at which the catalytic reaction is carried out depends primarily upon the nature of the transformation desired which in turn depends upon the nature of the stock. For example, when converting naphthene hydrocarbons into aromatic hydrocarbons, I have found that the temperature of operation is higher than when converting olefin hydrocarbons to naphthenes or paraffins. Naphthene hydrocarbons may be converted into aromatic hydrocarbons by operating the catalytic process at a temperature preferably between 850° F. and 1000° F. although lower yields of aromatics per pass may be obtained at temperatures as low as 750° F. Temperatures above 1000° F. may be used particularly when the stock does not contain hydrocarbons that will cause undesirable side reactions such as the cracking of paraffins to produce olefins. Olefin hydrocarbons are converted to naphthenes and paraffins at temperatures preferably between 700° F. and 850° F., using the catalytic process of my invention although temperatures as low as 600° F. may be used with correspondingly lower yields of transformed materials. The olefin hydrocarbons may also be converted directly to predominantly aromatic hydrocarbons with some paraffin and naphthene formations by operating the catalytic process at temperatures above 850° F. The paraffin hydrocarbons may be converted to olefins by carrying out the catalytic reaction at temperatures above 900° F.

Thus, when treating hydrocarbon mixtures by the catalytic process of my invention, I may select and control temperatures suited to the stock to be treated and to the product desired. For example, when treating a hydrocarbon mixture consisting predominantly of naphthenes and paraffins, I may catalytically treat this stock at temperatures between 850° and 900° F. to convert all of the naphthenes into aromatics without appreciably altering the paraffins. When treating a mixture of hydrocarbons consisting predominantly of olefins and naphthenes, I may select a temperature for the reaction of about

750° to convert the olefins into naphthenes and paraffins without substantially changing the naphthenes into aromatics but by operating at temperatures between 850°-900° F., I may convert both the olefins and naphthenes into predominantly aromatics with some paraffin formation. Some naphthenes may be unchanged depending upon the rate of flow of material through the reactor. When treating a mixture of hydrocarbons consisting predominantly of olefins and paraffins, I may catalytically treat at about 750° F. and obtain transformation of olefins into naphthenes and paraffins without affecting the paraffins present in the charge. However, by increasing the temperature of reaction to 850-900° F., the olefins may be transformed directly into aromatics but the paraffins again will be substantially unchanged.

Pressure influences the reaction in that it reduces the time of the reaction and increases the catalytic activity of the catalyst to reduce the olefin content in the charging stock passing through the reactor. The process, however, may be carried out successfully at atmospheric pressure. I have obtained successful deolefination of hydrocarbons by employing pressures from atmospheric to 200 lbs. per square inch. Pressures from sub-atmospheric to as high as 5000 lbs. per square inch may be used. In the process of converting naphthenes to aromatics, superatmospheric pressure is not essential, in fact, in some cases, is detrimental since it reduces the yield of aromatics. However, by increasing the temperature of the reaction, the detrimental effect of pressure may be overcome.

In general, the process of transforming olefins and naphthenes is carried out by simply heating and vaporizing the stock to be treated to the desired reaction temperature, say 800° F., and passing the vapors through the reactor containing the catalyst and then condensing the products of the reaction. The reactor is preferably an elongated chamber containing the catalyst absorbed on granules of the suitable carrier. The reactor may be placed in either a horizontal, vertical or inclined position. In commercial operations, it may be desirable to provide a plurality of these reactors so that they may be operated alternately in order to provide for the removal and regeneration of the catalyst. If desired, the reactor may be provided with conveyors for containing the catalyst which may be moved through the reactor and out of the zone of reaction where the used catalyst may be reactivated or replaced with fresh catalyst before being introduced into the reactor. The variations of means and method for providing the catalyst in the reaction zone and for regeneration are obvious to those skilled in the art and form no particular part of my invention.

The products issuing from the reactor may be recycled through the reactor in cases where the passage of the stock through the reactor does not produce sufficient deolefination or desired transformation. Also, the rate of passage of the stock through the reactor, in other words, the reacting time, may be varied to give sufficient time for the feed in the reactor in order to obtain the desired reaction. By providing sufficient time in the reactor, the feed stock may be transformed adequately in a single passage through the reactor.

The condensed products of the reaction may then be treated to recover purer aromatic hy-

drocarbons. This may be accomplished by extracting the treated mixture with a solvent that selectively dissolves the aromatic hydrocarbons in the mixture and rejects as a fraction insoluble in the solvent the non-aromatic hydrocarbons such as the paraffin, naphthenic and other non-aromatic hydrocarbons. By allowing the mixture of treated material and solvent to stratify into two layers, the phase of solvent and aromatic fractions may be removed from the other phase of non-aromatic hydrocarbons and may then be distilled to recover the solvent. Solvents adapted to extract the aromatics from the non-aromatic hydrocarbons are liquid sulfur dioxide, phenol, dichlorethyl ether, furfural and the like.

The extraction of the treated hydrocarbons also extracts any residual olefins along with the aromatics. If desired, the extract containing the olefins may be retreated by the catalytic method to reduce further the olefins contained in the extract. The thus treated product may be re-extracted to remove non-aromatic hydrocarbons which may have been produced by the retreatment. This procedure of catalytic treatment and extraction may be repeated as many times as is necessary to produce an extract that is substantially free from olefins.

If desired, the original stock containing a mixture of hydrocarbons may be first extracted to separate and concentrate the olefins and aromatics present in the mixture and the extract may then be treated by the catalytic process to convert the olefins into non-olefinic materials. This, of course, will reduce the amount of stock to be passed through the catalyst reactor. If desired, the product obtained from the reaction may be treated with sulfuric acid to remove any traces of unconverted olefins.

While I have described above a particularly desirable use of my invention as applied to the purification of aromatic hydrocarbons to remove undesirable olefins, the process may be applied for the production of olefin-free, gum stable motor fuels of high anti-knock which may be used either per se or as a blend for other gasolines. For example, I may subject a pressure distillate composed chiefly of aromatics, paraffins and olefins to the above treatment and produce a motor fuel composed of aromatics, paraffins and naphthenes which is substantially free of olefins and which is superior to the original stock particularly with regard to stability to gum formation.

An aviation gasoline of high anti-knock may be produced from normally liquid olefins containing little or no aromatic hydrocarbons or non-olefinic material. This may be accomplished by subjecting the olefins to the catalytic treatment forming the subject matter of my invention to convert the olefins to a hydrocarbon fraction composed chiefly of naphthenes and having a knock rating, for example, of about 75-85 (A. S. T. M. Motor Method). By adding a small amount of tetra ethyl lead to this fraction, for example, 3 ml. per gallon of the gasoline, an aviation gasoline of 90-100 knock rating may be produced. The normally liquid olefins to be processed may be produced by polymerization of normally gaseous olefins.

It is thus another object of my invention to convert olefins into naphthenes to produce desirable motor fuels.

As stated above, the catalytic treatment of olefins converts these hydrocarbons into naph-

thenes which are at least partially converted into aromatic hydrocarbons. This is particularly true when using a catalyst of phosphoric acid which has been partially neutralized on the carrier with caustic soda. Instead of treating olefins to produce aromatic hydrocarbons, I may treat naphthene hydrocarbons by the above described catalytic method to produce aromatic hydrocarbons which may be extracted if desired to produce aromatic solvents.

I have also discovered that a motor fuel of suitable boiling range containing naphthene hydrocarbons may be catalytically treated as above to produce a motor fuel of improved anti-knock value. In this treatment, the naphthene hydrocarbons are converted into aromatic hydrocarbons which are of higher knock rating than the corresponding naphthenes. The presence of olefins in the charging stock is not essential as long as the gasoline contains naphthene hydrocarbons. For example, I may catalytically treat a gasoline fraction having an anti-knock value of about 65 and containing about 30% naphthene hydrocarbons and produce a motor fuel having an anti-knock value of about 75. This process may be operated on straight naphthenes, i. e. containing little or materially no other hydrocarbons or the treatment may be carried out on a mixture of naphthenes and aromatic or paraffinic or other hydrocarbons. When treating a straight naphthene fraction, for example, one containing cyclohexane, methyl cyclopentane, cycloheptane and substituted cyclo paraffins and having, for example, an anti-knock value of about 65, I may convert by the above catalytic treatment this fraction into one having a blending anti-knock value of about 100 and above which may be blended with gasolines of lower anti-knock values.

As stated above, the transformation of olefins to naphthenes and paraffins takes place at lower temperatures than the transformation of naphthenes to aromatics. I have discovered that olefins may be converted to aromatics by carrying the process in several stages of operation in which the temperature in each stage is controlled such that the olefins are first converted into naphthenes and paraffins in the first stage and the thus produced naphthenes are converted in the second stage into aromatics. Thus, by employing temperatures of 700-850° F. in the first stage, the olefins may be converted into naphthenes and paraffins and by employing temperatures above 850° F. in the second stage, the naphthenes may be converted into aromatics. The same type catalyst may be employed in each stage. While as shown previously, the olefins may be converted directly into aromatics in a single stage by operating at temperatures above 850° F., the two stage process has the advantage of less loss of material due to formation of gases as this process is carried out at lower temperatures.

When treating stocks that are predominately naphthenes and paraffins containing little or no olefins and it is desired to obtain the maximum production of aromatics from this stock, the first stage may be operated at higher temperature, i. e., above 900° F. This high temperature first stage operation will convert the naphthenes into aromatics and will convert the paraffins into olefins. The products of the first stage may then be passed through a second stage maintained at a lower temperature, i. e. 850° F.-900° F. in order to obtain transformation of the

olefins formed in the first reaction zone into aromatics. By recycling a part of the products from the second stage, a product may eventually be produced consisting of any desired aromatic content. The above two-stage operation wherein the first stage is operated at a higher temperature, i. e. above 900° F., then the second stage may be used to treat stocks that are predominately paraffins to produce aromatics. This may

10 be accomplished first by converting paraffins to olefins in the first stage and converting the olefins to aromatics in the second stage and recycling a part of these products to obtain a product of any desired aromatic content.

15 In the aforementioned two-stage operation, the charging stock may be either normally liquid or normally gaseous olefins and/or paraffins to produce the normally liquid aromatics, paraffins, naphthenes and olefins.

20 The two-stage catalytic process which is included within the scope of my invention is particularly suited for the reforming of low anti-knock gasolines to produce high anti-knock gasolines. Thus, I may subject gasoline containing appreciable quantities of naphthenes and low 25 knock rating paraffins to the catalytic treatment in the first stage operated at a relatively high temperature, i. e. above 900° F., to transform paraffin hydrocarbons into olefins and naphthenes

30 into aromatics. The products of the first reaction stage may then be passed through a catalytic zone maintained at a lower temperature, i. e. 850-900° F. to transform the olefins into aromatics.

35 Other objects, features and advantages of my invention will become apparent to those skilled in the art from the following specific examples:

#### EXAMPLE 1

40 A cracked gasoline was topped to produce a bottoms fraction having a boiling range of 200-450° F. and containing about 29.2% by weight of olefins. These bottoms were vaporized and the vapors were passed through a reactor 45 consisting of an elongated stainless steel tube about 4 feet long and about one inch in diameter which contained about 230 ml. of catalyst composed of phosphoric acid adsorbed on Columbia activated carbon. The topped gasoline 50 was passed through the reactor at a rate of about 125 ml. per hour. The temperature was maintained in the reactor at about 800° F. Atmospheric pressure was maintained throughout the operation. Water at a rate of 30 ml. per hour 55 was pumped into the vaporized stream of charging stock passing to the reactor. The hydrocarbon vapors and steam passing through the reactor were condensed and the water was removed from the hydrocarbons. The condensate 60 of hydrocarbons was again topped to remove fractions having a boiling point below 200° F. The catalyst was prepared by saturating carbon particles capable of passing through a screen of 6 mesh and being held on a 14 mesh screen, with 65 85% phosphoric acid and allowing the excess acid to drain from the carrier which was then dried at 400° F. About 230 ml. of the thus prepared catalyst was used to effect the reaction.

70 Tests on hourly samples of the recovered products of reaction boiling between 200-450° F. showed a consistent olefin content of about 13% which was maintained for at least 7 hours. The product of reaction containing 13% olefins was 75 recycled through the reactor containing the same

catalyst while maintaining the same operating conditions. The treated product from the reactor was again topped to 200° F. initial boiling point. A test on the bottoms showed a reduction in olefin to approximately 6.5%. The sulfur content of this product was reduced from 0.68% by weight contained in the original untreated material to 0.13%. The catalyst was further used to treat original feed for approximately 40 additional hours and the tests on the products passing through the reactor still showed a reduction of about 50% of olefins per cycle of charging stock.

#### EXAMPLE 2

A hydrocarbon fraction having a boiling range of 170-400° F. and composed of 60% by volume of aromatic hydrocarbons consisting chiefly of benzene, toluene and xylene, 14% by volume of olefins and 26% by volume of paraffins and other non-aromatic and non-olefinic hydrocarbons was treated with catalyst at 800° F. as in Example 1. After the first cycle of operation, the product of reaction showed an olefin content of 5.6%. This was reduced to 3.2% by recycling the once treated product through the reactor containing the catalyst under the same conditions of operation.

The liquid products of the reaction were then mixed with 2 volumes of liquid sulfur dioxide at a temperature of about -18° F. and the mixture was allowed to stratify into two layers consisting of an upper layer of non-aromatic hydrocarbons dissolved in a small amount of the sulfur dioxide and a lower layer consisting of the aromatic hydrocarbons dissolved in the bulk of the liquid sulfur dioxide. The lower layer was withdrawn and the liquid sulfur dioxide was distilled to produce a fraction of aromatic hydrocarbons and representing about 65% by volume of the material undergoing extraction. The extracted aromatics contained the small amount of unconverted olefins which were present in the treated stock and which were extracted along with the aromatics.

#### EXAMPLE 3

A pressure distillate was topped to produce a hydrocarbon fraction having a boiling range of 196-410° F. and composed of 20% olefins, 15% aromatics, 48% naphthenes and 17% paraffins. This fraction was then passed through the reactor containing 230 ml. of catalyst at a temperature of about 800° F. and atmospheric pressure and at a rate of 60 ml. per hour and was continued for five hours. The catalyst was prepared by adsorbing 25 ml. of 75%  $H_3PO_4$  on 230 ml. of

Columbia activated carbon of 6-14 mesh and stirring until dry without added heat. Then 25 ml. of 20% aqueous sodium hydroxide was added to the carbon containing the phosphoric acid and the mixture was stirred well while drying with the application of gentle heat. The amount of caustic soda added to the carbon containing the phosphoric acid represented one-half equivalent of the alkali per mol of the acid.

10 The total product recovered at the end of five hours of operation from the reactor which represented 93% of the feed charged to the reactor consisted of a hydrocarbon fraction having a boiling range of 170-429° F. and consisted of 2% olefins, 37% naphthenes, 26% aromatics and about 35% paraffins which was obtained in a single pass through the reactor. Very little gas was produced during the treatment and this consisted of 58.4% hydrogen, 1.4% olefins, 35.6% paraffins and 4.6% of material soluble in caustic soda.

15 The above treatment was retreated using the same feed stock, temperatures, pressure and catalysts in which the phosphoric acid adsorbed on the carbon was partially neutralized by various equivalents of caustic soda per mol of the phosphoric acid. The following table contains a summary of the catalyst used and the composition of the resulting product together with the gravity and Engier distillation of the final product. Included also are tests on the feed stock which was subjected to the treatment.

20 The product obtained by the treatment of the stock with phosphoric acid neutralized with one-half equivalent of caustic soda per mol of acid and having a composition of 2% olefins, 26% aromatics, 37% naphthenes and 35% paraffins was retreated using the same catalyst but at a higher temperature, i. e. 850-900° F. The resulting product which represented about 94% of the once treated feed stock showed an aromatic content of 65%, a paraffin content of 33% and an olefin content of 2% indicating that all of the naphthenes were converted into aromatics.

45

#### EXAMPLE 4

The polymer gasoline having a boiling range of 80-390° F. and composed of approximately 80% olefins and 20% paraffins was treated in accordance with Example 3 using the phosphoric acid catalyst which had been neutralized with one-half equivalent of caustic soda per mol of acid. The treated product representing 92% by volume of the feed stock and obtained in a single pass through the reactor consisted of 5% olefins, 15% aromatics, 12% naphthenes and 68% paraffins.

Table 1

| Catalyst used— $NaOH$ per mol of $H_3PO_4$ on activated carbon | Composition of treated product, per cent by volume |           |            |           | Gravity<br>A. P. I.<br>at 60° F. | Engier distillation, °F. |     |     |     |         |
|----------------------------------------------------------------|----------------------------------------------------|-----------|------------|-----------|----------------------------------|--------------------------|-----|-----|-----|---------|
|                                                                | Olefins                                            | Aromatics | Naphthenes | Paraffins |                                  | Initial                  | 10% | 50% | 90% | Maximum |
| No equivalent                                                  | 7                                                  | 19.0      | 45.0       | 29.0      | 48.0                             | 180                      | 227 | 297 | 373 | 429     |
| 1/4 equivalent                                                 | 2.4                                                | 20.4      | 35.1       | 32.1      | 47.8                             | 188                      | 229 | 299 | 370 | 423     |
| 1/2 equivalent                                                 | 2.4                                                | 22.0      | 35.0       | 34.6      | 47.4                             | 160                      | 230 | 290 | 370 | 429     |
| 1/4 equivalent                                                 | 2.0                                                | 21.0      | 37.0       | 34.0      | 47.6                             | 170                      | 227 | 296 | 372 | 429     |
| 1/2 equivalent                                                 | 2.6                                                | 23.0      | 34.0       | 34.5      | 47.5                             | 171                      | 229 | 293 | 371 | 429     |
| 1/4 equivalent                                                 | 4.5                                                | 21.0      | 40.5       | 34.0      | 47.8                             | 172                      | 228 | 290 | 373 | 421     |
| 1 equivalent                                                   | 5.2                                                | 20.8      | 41.5       | 33.0      | 47.7                             | 171                      | 220 | 290 | 371 | 421     |
| 1 1/2 equivalent                                               | 5.0                                                | 21.0      | 41.0       | 32.0      | 47.8                             | 171                      | 220 | 290 | 372 | 421     |
| 2 equivalent                                                   | 5.1                                                | 19.0      | 45.0       | 27.9      | 48.0                             | 183                      | 226 | 290 | 375 | 420     |
| 3 equivalent                                                   | 18.3                                               | 17.0      | 45.0       | 23.8      | 48.2                             | 188                      | 240 | 301 | 374 | 415     |
| Composition and tests on feed stock                            | 20.0                                               | 15.0      | 45.0       | 17.0      | 48.5                             | 196                      | 243 | 303 | 376 | 410     |

## EXAMPLE 5

A straight run gasoline was extracted with 2 volumes of liquid sulfur dioxide at 18° F. to produce an extract consisting of 50% aromatics, 30% naphthenes and 20% paraffins. This fraction was catalytically treated at 850-900° F. and atmospheric pressure as in Example 3, using the phosphoric acid catalyst neutralized with one-half equivalent of caustic soda per mol of the acid. The treated product obtained in a single pass through the reactor and representing about 92% by volume of the feed stock introduced into the reactor consisted of 80% aromatics and 20% paraffins. The gravity and Engler distillation of the extract feed stock and the final product are given below:

Table 2

|                       | Gravity<br>° A. P. I.<br>at 60° F. | Engler distillation, °F. |     |     |     |     |      |
|-----------------------|------------------------------------|--------------------------|-----|-----|-----|-----|------|
|                       |                                    | Initial                  | 10% | 50% | 90% | 95% | Max. |
| Gasoline extract feed | 41                                 | 213                      | 247 | 282 | 335 | 352 | 382  |
| Final product         | 37                                 | 164                      | 233 | 271 | 319 | 343 | 396  |

## EXAMPLE 6

A pressure distillate was topped to produce a hydrocarbon fraction having a boiling range of 200-400° F. and was composed of 44% olefins, 10% aromatics, 20% naphthenes and 26% paraffins. This fraction was then passed through a reactor consisting of an elongated stainless steel tube about four feet long and about one inch in diameter which contained 230 ml. of catalyst at a temperature of about 750-800° F. and atmospheric pressure and at a rate of 60 ml. per hour. The catalyst was prepared by adsorbing 75 ml. of an aqueous solution of 20 ml. of sodium silicate solution diluted with 55 ml. of water on 230 ml. of Columbia activated carbon. The sodium silicate solution was the Philadelphia Quartz Company's E Brand sodium silicate solution of 40° Baumé and having an alkali-silica ratio of 1 to 3.22. The approximate composition of this sodium silicate solution is 29% SiO<sub>2</sub>, 9% Na<sub>2</sub>O and 62% H<sub>2</sub>O. Then the activated carbon containing the sodium silicate solution was allowed to soak in 500 ml. of 3N-HCl for about two days with occasional stirring. The excess hydrochloric acid was then drained from the granules of the carbon and these were washed thoroughly with water to remove free sodium chloride and hydrochloric acid before use, leaving a surface of silicic acid on the carbon granules. The granules are then dried at 300° F. The drying and the use of the catalyst at more elevated temperatures causes the silicic acid to gradually change to silica so that the major catalytic operation is with silica on the activated carbon.

## EXAMPLE 7

A straight run gasoline having a boiling range of 190-380° F. and composed of 14% aromatics, 42% naphthenes, 43% paraffins and 1% olefins and having an octane number of 60 was passed through a reactor containing about 4 liters of the catalyst described in Example 6 at a temperature of 850° F. and atmospheric pressure. The rate of passage of the gasoline through the reactor was 750 ml. per hour. The total product recovered from the reactor at the end of 14 hours of operation consisted of a hydrocarbon fraction having a boiling range of 170-360° F. and consisted of 30% aromatics, 25% naphthenes, 40% 75

paraffins and 4% olefins and had an octane number of 75.

The foregoing description is not to be taken as limiting my invention but merely as illustrative of one mode of carrying it out as many variations may be made thereon as will be recognized by those skilled in the art which are within the scope of the following claims.

I claim:

- 10 1. A catalyst comprising the product of a mixture of a carrier and an acid containing a phosphate radical, said catalyst being prepared by adsorbing phosphoric acid on said carrier followed by neutralizing said phosphoric acid on said carrier with approximately one-sixth to two-thirds equivalents of a caustic alkali per mol of said acid.
- 15 2. A catalyst comprising the product of a mixture of carbon and an acid containing a phosphate radical, said catalyst being prepared by adsorbing phosphoric acid on said carbon followed by neutralizing said phosphoric acid on said carbon with approximately one-sixth to two-thirds equivalents of a caustic alkali per mol of said acid.
- 20 3. A catalyst comprising the product of a mixture of activated carbon and an acid containing a phosphate radical, said catalyst being prepared by adsorbing phosphoric acid on said activated carbon followed by neutralizing said phosphoric acid on said activated carbon with approximately one-sixth to two-thirds equivalents of a caustic alkali per mol of said acid.
- 25 4. A catalyst according to claim 1 in which the carrier is alumina.
- 30 5. A method of preparing a catalyst which comprises adsorbing phosphoric acid on a carrier and subsequently neutralizing said phosphoric acid on said carrier with approximately one-sixth to two-thirds equivalents of a caustic alkali per mol of said acid.
- 35 6. A method of preparing a catalyst which comprises adsorbing phosphoric acid on carbon and subsequently neutralizing said phosphoric acid on said carbon with approximately one-sixth to two-thirds equivalents of a caustic alkali per mol of said acid.
- 40 7. A method of preparing a catalyst which comprises adsorbing phosphoric acid on activated carbon and subsequently neutralizing said phosphoric acid on said activated carbon with approximately one-sixth to two-thirds equivalents of a caustic alkali per mol of said acid.
- 45 8. A method as in claim 5 in which the carrier is alumina.
- 50 9. A method of preparing a catalyst which comprises adsorbing phosphoric acid on a carrier, drying the mixture and subsequently neutralizing said phosphoric acid on said carrier with approximately one-sixth to two-thirds equivalents of a caustic alkali per mol of said acid.
- 55 10. A method of preparing a catalyst which comprises adsorbing phosphoric acid on carbon, drying the mixture and subsequently neutralizing said phosphoric acid on said carbon with approximately one-sixth to two-thirds equivalents of a caustic alkali per mol of said acid.
- 60 11. A method of preparing a catalyst which comprises adsorbing phosphoric acid on activated carbon, drying the mixture and subsequently neutralizing said phosphoric acid on said activated carbon with approximately one-sixth to two-thirds equivalents of a caustic alkali per mol of said acid.

KARL KORPI.